

Feb. 16, 1932.

H. BOVING

1,845,041

INSULATED ELECTRIC CONDUCTOR

Filed Sept. 16, 1927

FIG. 1



FIG. 2



INVENTOR  
HENRIK BOVING  
By Walter C. Kiesel  
ATTORNEY

## UNITED STATES PATENT OFFICE

HENRIK BOVING, OF NEW YORK, N. Y., ASSIGNOR TO BELL TELEPHONE LABORATORIES,  
INCORPORATED, OF NEW YORK, N. Y., A CORPORATION OF NEW YORK

## INSULATED ELECTRIC CONDUCTOR

Application filed September 16, 1927. Serial No. 219,908.

This invention relates to the insulation for electrical conductors. One application of it is in insulating wire and more particularly to the insulating of copper wire of the type 5 having a coating of baked enamel.

When the usual types of enamels, such as black compound and varnish enamels, are applied and baked directly on tinned copper wires, the enamel adheres so firmly to the 10 wire that it is difficult to remove unless it is baked very soft or very hard. Either the very soft or the very hard baking of the enamel coating is undesirable because in the very soft state the coating is susceptible to 15 mechanical injury and in the very hard state it becomes brittle and will not stand handling or bending without flaking. Furthermore, in the case of tinned copper wire the baking incident to producing a very hard 20 enamel coating causes the tin to partly alloy with the copper, thereby producing a surface which is difficult to solder.

The invention in one aspect consists of means between the enamel insulation and the 25 conductor for facilitating the removal of the insulation.

In a more specific aspect, the invention comprises applying to a tinned wire a priming coating of adhesive material, such as a 30 varnish containing a phenolic condensation product, or a varnish composed of a metallic soap dissolved in a volatile solvent, baking the coating to form an adherent layer, applying to the priming coating a coating of insulating 35 enamel and baking the double coating at a higher temperature than the baking temperature of the priming coating, to change the priming coating to a substantially non-adherent layer and form an insulation having the necessary qualities of flexibility, inertness to solvents and freedom from embrittling upon aging. The thin priming coating has the property of being more adherent to the insulating enamel than to the 40 surface of the wire so that the insulation may be easily and completely removed by stripping, by mechanical means, thus leaving the tinned wire in suitable condition for soldering purposes.

50 A more detailed description of the inven-

tion follows and is illustrated in the accompanying drawings.

Fig. 1 illustrates a conductor having a thin priming coating of material which is substantially non-adherent and an outer coating of 55 elastic insulating enamel.

Fig. 2 is a cross-sectional view of Fig. 1.

Referring to the drawings, Fig. 1 shows an electrical conductor 10, of copper, having a thin coating of tin to form a surface which 60 is easy to solder. The amount of tin in the coating is necessarily small being approximately from one to six milligrams per square inch of conductor surface. Heavy tin coatings are not suitable for subsequent enameling because the enamel coating is usually baked at a temperature above the melting point of tin, and heavy coatings produce a sufficient amount of liquid tin in the enamel baking process so that the tin collects in droplets under the enamel applied to the conductor. A thin priming coating 11 is applied to the tinned conductor or wire 10 and is 65 preferably of an adhesive material which can be baked to a hard non-adherent state at a 70 temperature not greater than that used for producing the usual type of enamel coating in the adherent flexible state.

It has been found that varnishes containing a condensation product of the phenol 80 group, such as "bakelite" varnishes, or a varnish or enamel prepared by dissolving metallic soaps in boiled vegetable oils are suitable for the priming coat. By diluting the varnish or enamel with a suitable volatile 85 solvent, the thickness of the priming coating may be varied from .0002 of an inch to .00005 of an inch. A desirable varnish of the metallic soap type may be produced by dissolving aluminum linoleate in linseed oil which 90 has been boiled to varnish consistency.

After the priming coating has dried sufficiently to form a hard adherent layer, a covering or coating 12, preferably of insulating enamel is applied thereto in any suitable manner and the insulated conductor is treated to produce a coating of the desired flexibility and hardness. After this treatment which is 95 preferably accomplished by baking at a suitable temperature, the priming coating be-

comes non-adherent and adheres more firmly to the insulating enamel than to the surface of the conductor.

The preferred method of producing an insulating enameled coating which may be easily stripped from the conductor comprises, applying a coating or coatings of the priming varnish and baking the coating at a temperature between 300° and 400° F. to form a sufficiently flexible adherent layer which will not crack or flake off during the subsequent enameling process. When the priming coating consists of a varnish containing a phenolic condensation product, the baking temperature should be approximately 400° F., while the baking temperature of the metallic soap varnish should be approximately 500° F. This preliminary baking temperature can be changed, however, depending upon the type of varnish used in the priming coat since the object of this baking is to dry the varnish and produce sufficient adherence of the varnish to the conductor during subsequent operations. The conductor is passed through a bath containing an enamel in any suitable manner to form a layer or a plurality of layers of protective insulation and finally baked at a suitable temperature from approximately 500° to 600° F. The enameling and baking may be performed in a continuous operation in an oven structure such as is disclosed in the Holmes and Harris Patent 1,101,281, dated June 23, 1914.

The final baking temperature which is higher than the baking temperature of the priming coating changes the priming coating from a flexible adherent layer to a substantially non-adherent coating on the conductor surface. The priming coating is of a fragile character but due to its adherence to the enamel insulation the two coatings may be easily stripped from the conductor by mechanical means, such as pliers, and the tinned conductor will be in clean condition for soldering operations.

By regulating the thickness of the priming coating, enamel coatings may be produced varying from the condition of being very adherent and therefore difficult to remove, to the condition of being quite non-adherent, easy to remove and simulating a tube of insulation. The thicker coating allows the enamel to be removed from the core or wire as hollow flexible insulation by stretching the wire in a well known manner or by reducing the diameter of the wire. This hollow flexible insulation forms the subject matter of my divisional copending application, Serial No. 395,171, filed September 25, 1929.

The invention is not limited to the specific materials mentioned for the priming coating since other materials may be employed which would become non-adherent continuous priming layers after the insulating coating has been applied and treated as described above.

Furthermore, the invention is not limited to the particular method of baking since the coatings may be treated by other media to cause the priming coating to become non-adherent to the conductor.

What is claimed is:

1. The method of forming a coating of insulation on an electric conductor which comprises, applying to the conductor a coating of adhesive material, applying thereto a coating of insulation, and treating the insulated conductor to render the inner coating non-adherent. 70

2. The method of forming a coating of insulation on an electric conductor which comprises, applying to the conductor a coating of adhesive material, applying thereto a coating of insulation, and applying heat to the insulated conductor to render the inner coating non-adherent. 75

3. The method of forming a coating of insulation on an electric conductor which comprises, applying to the conductor a coating of varnish, applying thereto a coating of insulation, and treating the insulated conductor to render the inner coating non-adherent. 80

4. The method of forming a coating of insulation on an electric conductor which comprises, applying to the conductor a coating of varnish, applying thereto a coating of insulation, and applying heat to the insulated conductor to render the inner coating non-adherent. 85

5. The method of forming a coating of insulation on an electrical conductor which comprises, applying to the conductor a coating of adhesive material, applying thereto a coating of insulating enamel, and treating the insulated conductor to render the inner coating non-adherent. 90

6. A method of forming a coating of insulation on an electrical conductor which comprises, applying to the conductor a coating of adhesive material, applying thereto a coating of insulating enamel, and applying heat to the insulated conductor to render the inner coating non-adherent. 95

7. The method of forming a coating of insulation on an electric conductor which comprises, applying to the conductor a coating of varnish, applying thereto a coating of insulating enamel, and applying heat to the insulated conductor to render the inner coating non-adherent. 100

8. The method of forming a coating of insulation on a conductor which comprises, applying to the conductor a priming coating of insulating material which is adherent when dried and becomes non-adherent when heated a sufficient amount, applying a second coating of a different insulating material, and heating the two coatings to render the priming coating non-adherent. 105

9. The method of forming a coating of insulation on a conductor which comprises, ap- 110

- plying a coating of varnish having properties which change within a certain range of temperatures, baking the coating at temperatures between 300° and 500° F., applying a finishing coating of elastic material, and baking the two coatings at temperatures between 500° and 600° F. 70
10. The method of forming a coating of insulation on a conductor which comprises, applying a varnish containing a phenolic condensation product, baking the varnish at a temperature of approximately 400° F., applying an insulating enamel to said varnish, and baking the varnish and enamel at a temperature of approximately 600° F. 80
11. An electric conductor insulated with baked enamel, comprising a layer in contact with the conductor for spacing the insulation from the conductor, said layer being non-adherent to the conductor. 85
12. An electric conductor insulated with baked enamel, comprising a layer of fragile varnish between the enamel and the conductor for facilitating the removal of the insulation. 90
13. An electric conductor insulated with baked enamel, comprising a phenolic condensation varnish between the insulation and the conductor for preventing the latter adhering firmly to the former. 95
14. An electric conductor insulated with baked enamel, comprising a layer of varnish containing an embrittling agent between the enamel and the conductor for preventing the adherence of the enamel to the conductor. 100
15. An insulated conductor having a plurality of coatings of insulating material thereon, the innermost coating consisting of a thin priming layer of varnish, said layer being substantially non-adherent to the surface of the conductor and firmly adherent to the adjacent coating of insulating material. 105
16. An insulated conductor comprising a central wire having a non-adherent priming layer of varnish containing a phenolic condensation product, and an outer coating of insulating enamel firmly adherent to said non-adherent priming layer. 110
17. The method of forming a coating of insulation on a conductor which comprises applying a varnish to the conductor containing a material which is non-adherent when heated to a certain temperature, baking the coating at a temperature to dry the varnish on the conductor, applying an insulating enamel to said coating, and baking the varnish and enamel at a temperature of approximately 600° F. 115
18. The method of forming a coating of insulation on a conductor which comprises applying to the conductor a priming coating of insulating material which changes from an adherent to a non-adherent state within a certain range of temperatures, baking the priming coating at a temperature below the 120
- transition temperature, applying a second coating of a different insulating material, and baking the two coatings at a temperature higher than the transition temperature of said priming coating. 125
19. The method of forming a coating of insulation on a conductor which comprises applying a coating of varnish having properties which change at high temperatures, baking the coating to form an adherent layer, applying a finishing coating of elastic material, and baking the two coatings at a higher temperature than the first baking temperature, whereby the varnish coating adheres to the finishing coating more firmly than to the conductor. 130
20. In an insulated conductor, a layer of insulating varnish adjacent to the bare conductor composed of material which is substantially non-adherent thereto, and a layer of insulating enamel adherent to said varnish, said layers being capable of being easily stripped from the conductor. 135
- In witness whereof, I hereunto subscribe my name this 8th day of September, A. D. 1927.
- HENRIK BOVING.